

# UNITED STATES PATENT OFFICE.

CHARLES MOTIER NES, OF YORK, PENNSYLVANIA.

## IMPROVEMENT IN REWORKING BESSEMER STEEL.

Specification forming part of Letters Patent No. 102,960, dated May 10, 1870. .

*To all whom it may concern:*

Be it known that I, CHARLES MOTIER NES, of York, in the county of York, and State of Pennsylvania, have invented certain new and useful Improvements in Reworking Scrap, Old Rails, Imperfect Ingots, &c., of Bessemer Steel, and of converting the same into malleable iron, cast-steel, or puddled steel, of which the following is a specification:

In the manufacture of Bessemer steel it is usual to decarbonize the iron by means of blast, and then decarbonize it by the addition of spiegeleisen, a highly-carbonized pig-iron, which is thrown in sufficient quantities to produce steel.

The Bessemer steel thus made, on account of the quantity of carbon it contains, cannot be reworked.

The ordinary way of reworking old iron rails is by piling and rerolling. This is not practicable with the Bessemer-steel rails, as the pile will not weld on account of the carbon contained in the metal; and, again, if it be desired to puddle the Bessemer steel in the ordinary way, the metal cannot be balled up, and even if it could be it would fly under the hammer, this being due to the carbon which it contains.

It is owing to this fact that old and imperfect steel rails, ingots, scrap, &c., in large quantity, are allowed to go to waste, no plan having yet been devised by which to rework them advantageously and profitably.

The object of my invention is to utilize this waste material, and to rework it into malleable iron, cast-steel, or puddled steel, simply, cheaply, and expeditiously. To this end I employ the following process, the first essential condition of which is to deprive the Bessemer metal of the carbon with which it is charged:

I first melt the old rails, ingots, or other articles of Bessemer steel to be reworked in an ordinary cupola, employing a hot or cold blast, as desired. When the metal is melted, I run it from the cupola into a refining-furnace, which I prefer to make of cast-iron plates lined with fire-brick. Two or more tuyeres are provided on either side of this furnace, and, after the metal is run therein, air or oxygen is blown through the tuyeres into the

melted mass until the carbon is thoroughly eliminated from the metal.

If, however, it is desired to produce cast-steel, I conduct the melted and decarbonized metal from the refining-furnace through a "run-out," usually employed with such furnaces, into an air-tight chest or receptacle, such, for instance, as described in my patent dated April 19, 1870, where the metal is re-carbonized by blowing carbonized gases into the chest, or by throwing sufficient pig-iron into the metal, following substantially the process described in said patent.

In this manner I obtain steel which can be run from the chest into molds of any shape and size desired, and can be thence taken and put under the hammer and made into rails of quite as good quality as the Bessemer rails when first made.

In order to repuddle the steel, I take the melted metal from the refining-furnace, after it has been deprived of its carbon by the process above specified, and run it into the puddling-furnace, where it is puddled in the ordinary way, a sufficient quantity of pig-iron and silica being employed to keep a bath over the iron, thus keeping carbon enough in the pig to reconvert it into steel.

I prefer, in order to hasten the process, and to produce finer metal, to insulate both the cupola or melting-furnace and the refining-furnace, and to insert into the melted metal steel bars, which are connected with a galvanic battery, as described in my patent above named, thus causing continued currents of electricity to traverse the metal while it is melting and refining.

Electricity may also be employed with the re-carbonizing process, if desired, although the use of electricity is not indispensable in any of the stages of the process.

Having now described my invention, and the manner in which the same is or may be carried into effect, what I claim, and desire to secure by Letters Patent, is—

1. The method of producing malleable iron from old rails, imperfect ingots, scrap, &c., of Bessemer steel, substantially in the manner herein specified.

2. The manufacture of cast-steel from old rails, imperfect ingots, &c., of Bessemer steel,

by first melting and decarbonizing the metal to be reworked, and then recarbonizing the same, substantially in the manner described.

3. The manufacture of puddled steel from imperfect ingots, scrap, &c., of Bessemer steel, substantially in the manner described.

In testimony whereof I have signed my

name to this specification before two subscribing witnesses.

**CHAS. MOTIER NES.**

Witnesses:

**JOHN A. WILSON,**

**IVAN GLOSSBRENNER.**